

## UNITED STATES PATENT OFFICE

NEIL MACCOULL, JR., OF ENGLEWOOD, NEW JERSEY, ASSIGNOR TO THE TEXAS COMPANY, OF NEW YORK, N. Y., A CORPORATION OF DELAWARE

## LUBRICATING OIL

No Drawing.

Application filed August 15, 1928. Serial No. 299,881.

This invention relates to lubricating oils suitable for the lubrication of internal combustion engines and particularly to a lubricant adapted to substantially maintain its viscosity during use and to adequately lubricate the engine parts.

It is a common observation that the lubricating oil used in a recirculating system of a conventional internal combustion engine, employing commercial liquid fuels, such as gasoline or kerosene, becomes diluted with the fuel. This effects a reduction in the viscosity of the oil and depreciates its value as a lubricant. It has also been observed that this contamination continues at a decreasing rate until a state of equilibrium is reached, after which the viscosity of the oil in the crank case remains substantially constant. Under this latter condition the rate of evaporation of the fuel dissolved in the oil is believed to be substantially equal to the rate at which the fuel passes the pistons of the engine and enters the lubricating oil. This rate of evaporation would increase with the concentration of the fuel in the oil and with the temperature of the crank case. In other words, one method for controlling the extent of dilution of the lubricating oil with fuel is to maintain the crank case of the engine at a selected temperature. Observations bearing on these facts have been disclosed and proven by experiments described in an article entitled "Consumption and dilution of automobile engine oils", S. A. E. Journal, July, 1924, by Neil MacCoul.

Unfortunately, this "equilibrium viscosity" is often too low for satisfactory lubrication of an engine, unless the oil used was originally of such high viscosity as to have interfered with the proper flow of oil in the lubricating system until it had been in service a sufficient length of time to have acquired a quantity of the fuel diluent. This is particularly true when an engine is first started during cold weather.

During investigations based on the foregoing premises, it has been found, therefore, that if an oil of high viscosity is brought into a state that corresponds approximately to the "equilibrium viscosity" before it is put

into an engine, the latter may be run for long periods with a comparatively uniform viscosity or at the most a very slightly declining viscosity.

A numberless variety of oils may be prepared in accordance with the foregoing suggestions, the broad principle of which consists in an oil prepared by blending a comparatively high viscosity lubricating oil with a low boiling distillate in such proportions that the viscosity of the blended oil experiences no sharp changes in use. In common with the usual motor oils, such blended oils are usually made with the object of attaining a desired viscosity. In order to provide thorough and efficient lubrication, it is desirable to incorporate in such blended oils a small amount of a material having exceptionally high lubricating value. An example of such material is a specially prepared oxidized paraffin wax which is substantially free from gummy and other materials insoluble in the blended motor oil. These oxidized hydrocarbons have been found to have exceptional lubricating properties and have been found in general to greatly improve the lubricating value of ordinary lubricating oils by blending a small amount of these oil-soluble oxidized hydrocarbons in them. Although I prefer to use the material derived from a limited oxidation of paraffin wax for incorporating with oil, other oxidized hydrocarbons of the paraffin series, particularly of the more complex higher boiling, highly viscous and semi-solid hydrocarbons may be employed.

In order to more fully illustrate my invention, but without limiting effect thereon, the following example is given:

A lubricating oil having a Saybolt viscosity of about 500 sec. at 100° F. may be prepared by blending a naphthalene base lubricating oil of about 1700 sec. Saybolt viscosity at 100° F. with a light distillate whose distillation range lies between about 310° F. and 420° F. in the proportion of about 91 parts by volume of heavy oil to 9 parts by volume of distillate. To this blended oil may be added a small proportion of oxidized paraffin wax in the proportion of about 2%. 100

Larger quantities of the oxidized wax may be used if desired but I prefer to use very small quantities since these have been proven sufficient to give the desired results. The oxidized wax will blend without difficulty in the lubricating oil and will not separate out even at comparatively low temperatures.

To facilitate the blending, however, it may be desirable to dissolve the oxidized wax in the light distillate prior to blending the distillate with the heavy oil. An oil blended as thus indicated, will have a flash point of about 185° F. and a Saybolt viscosity of about 500 sec. at 100° F.

For the preparation of a lubricating oil having a Saybolt viscosity of 300 sec. at 100° F., I may employ the same lubricating oil and the light distillate, but in the proportion of 88 parts by volume of lubricating oil to 12 parts by volume of the distillate containing the desired amount of oxidized paraffin wax. Such an oil will have a flash point of about 170° F.

The other standard viscosity engine lubricating oils may similarly be prepared by employing a lower or higher viscosity base lubricant or a lesser or greater amount of diluent. Satisfactory lubricants may be made in accordance with my invention by blending lubricating oils having a Saybolt viscosity as high as 3000 sec. with diluents boiling over a range from 300° F. to 500° F. and containing the desired amount of oxidized wax.

My new lubricant is to be distinguished from previously used motor oils containing oxidized paraffin wax and which may have acquired a certain dilution, as hereinbefore explained, by the dissolving of the fuel in the lubricant during use. I therefore employ in certain of the following claims the term "unused" to indicate this differentiation and the term is to be construed in the claims as here indicated.

Oxidized paraffin wax for blending may be prepared for example as follows:

A charge of crude scale paraffin wax, or if desired, more refined wax, is placed in an enamel or aluminum vessel which is preferably jacketed or otherwise fitted to permit accurate control of the temperature of the contents. Air is introduced in fine streams near the bottom of the heated wax maintained at temperatures between 260° and 330° F., preferably between 315° and 320° F. The oxidation is carried on until the acid value indicated by samples withdrawn for test is found to be about 35 and preferably not to exceed 40. Upon cooling this material, it will solidify and is found to have a light yellow color and when rubbed between the fingers has a greasy feeling.

If the oxidation has been carried out properly, the oxidized material will be found to be completely soluble in the previ-

ously mentioned light distillate and in the lubricating oil blend and will not deposit gummy or insoluble substances on standing.

Instead of employing paraffin wax as the starting material for oxidation, some of the heavier liquid or semi-liquid paraffin hydrocarbons may be employed after suitable refining and purifying treatment preferably with concentrated sulphuric acid. Liquid oils thus refined have been found to readily oxidize to produce materials similar in character to that derived from the oxidation of paraffin wax.

I am aware of previous suggestions to the use of lubricating oils blended with a light distillate as suggested in Wilson Patent No. 1,547,141, but by the use of my present invention superior results may be attained in the lubrication of internal combustion engines.

What I claim is:

1. An unused lubricating oil for internal combustion engines consisting of a lubricating oil having a viscosity equal to or higher than that normally used for the lubrication of internal combustion engines blended with a lesser amount of a hydrocarbon boiling below 500° F. and about 2% of oxidized paraffin wax, and having a relatively low decrease in viscosity during use.

2. An unused lubricating oil for internal combustion engines consisting of an oil having a viscosity of over 1000 sec. Saybolt at 100° F. blended with less than 25% by volume of a hydrocarbon oil boiling below 500° F. and about 2% of oxidized paraffin wax.

3. An unused lubricating oil for internal combustion engines characterized by having a flash point above 150° F., a Saybolt viscosity of at least 140 at 100° F., a relatively low loss in viscosity during use, and a content of between 7% and 15% of fractions boiling between about 300° F. and 460° F., and about 2% of oxidized paraffin wax.

4. An unused lubricating oil for internal combustion engines consisting of a lubricating oil having a viscosity equal to or higher than that normally used for the lubrication of internal combustion engines blended with a lesser amount of a hydrocarbon boiling below 500° F. and a small proportion of oxidized paraffin wax which is completely soluble therein, and having a relatively low decrease in viscosity during use.

5. An unused lubricating oil for internal combustion engines characterized by having a flash point above 150° F., a Saybolt viscosity of at least 140 at 100° F., a relatively low loss in viscosity during use, and a content of between 7% and 15% of fractions boiling between about 300° F. and 460° F., and a small proportion of oxidized paraffin wax which is completely soluble therein.

6. An unused lubricating oil for internal combustion engines consisting of a lubricat-

ing oil having a viscosity equal to or higher than that normally used for the lubrication of internal combustion engines blended with a lesser amount of a hydrocarbon boiling below 500° F. and less than 2% of oxidized higher paraffin hydrocarbons which are completely soluble therein, and having a relatively low decrease in viscosity during use.

10 In witness whereof I have hereunto set my hand and seal this 13th day of August, 1928.

NEIL MacCOULL.

#### CERTIFICATE OF CORRECTION.

Patent No. 1,767,147.

Granted June 24, 1930, to

NEIL MacCOULL, JR.

It is hereby certified that error appears in the printed specification of the above numbered patent requiring correction as follows: Page 2, lines 92 and 115, claims 1 and 4, and page 3, line 4, claim 6, after the word "hydrocarbon" insert the word "distillate"; and that the said Letters Patent should be read with these corrections therein that the same may conform to the record of the case in the Patent Office.

Signed and sealed this 9th day of September, A. D. 1930.

(Seal)

M. J. Moore,  
Acting Commissioner of Patents.

45

50

55

60

65

ing oil having a viscosity equal to or higher than that normally used for the lubrication of internal combustion engines blended with a lesser amount of a hydrocarbon boiling below 500° F. and less than 2% of oxidized higher paraffin hydrocarbons which are completely soluble therein, and having a relatively low decrease in viscosity during use.

10 In witness whereof I have hereunto set my hand and seal this 13th day of August, 1928.

NEIL MacCOULL.

#### CERTIFICATE OF CORRECTION.

Patent No. 1,767,147.

Granted June 24, 1930, to

NEIL MacCOULL, JR.

It is hereby certified that error appears in the printed specification of the above numbered patent requiring correction as follows: Page 2, lines 92 and 115, claims 1 and 4, and page 3, line 4, claim 6, after the word "hydrocarbon" insert the word "distillate"; and that the said Letters Patent should be read with these corrections therein that the same may conform to the record of the case in the Patent Office.

Signed and sealed this 9th day of September, A. D. 1930.

(Seal)

M. J. Moore,  
Acting Commissioner of Patents.

45

50

55

60

65